

March 8, 1938.

R. L. WAGNER

2,110,781

METHOD AND APPARATUS FOR CUTTING AND TREATING METALS

Filed Nov. 29, 1933



INVENTOR  
ROBERT L. WAGNER  
BY  
Sol Greenwald -  
ATTORNEY

## UNITED STATES PATENT OFFICE

2,110,781

METHOD AND APPARATUS FOR CUTTING  
AND TREATING METALSRobert L. Wagner, Astoria, N. Y., assignor, by  
mesne assignments, to Union Carbide and Car-  
bon Corporation, a corporation of New York

Application November 29, 1933, Serial No. 700,177

13 Claims. (Cl. 148—9)

This invention relates to the art of cutting metals, and more particularly to a method of preventing or removing certain objectionable metallurgical changes which are produced in 5 high carbon and alloy steels when they are severed by means of high temperature heating and oxidizing agents, e. g., the oxy-acetylene cutting flame, and allowed to cool undisturbed to atmospheric temperature.

10 When certain grades of steels are cut by the oxy-fuel gas process, the severed sections are ordinarily allowed to cool undisturbed to atmospheric temperature. The rate of cooling in air, supplemented by the heat conduction away from 15 the cut edges into the adjoining body portions of the sections, is sufficiently rapid to constitute an effective quench for the cut edges of high carbon and alloy steels in which a very marked and undesirable hardening usually takes place which is 20 due to the enhanced hardening properties of these steels. The hardened zone thus produced seldom extends beyond a fraction of an inch from the cut surface or edge but is sufficiently deep to reduce effectively the ductility and produce other 25 changes which limit the usefulness of sections of such steels when cut by the oxy-fuel gas process. This increase in hardness is accompanied by a decided embrittlement of the metal at the cut edges and makes these cut surfaces very difficult 30 to machine. This hardened zone also serves as a starting point for cracks which may propagate readily into the unaffected metal when mechanical or thermal stresses are present. These characteristics are particularly true of those grades of 35 steel (such as carbon steels containing above about 0.35% carbon, the structural silicon steels and some steel alloys containing nickel, chromium, manganese or vanadium) whose compositions are such as to impart to them the property 40 of air hardening when they are heated beyond their recrystallization temperature and allowed to cool rapidly in air,—conditions which are approached and/or duplicated in the severing of such metals by the ordinary practices of high- 45 temperature flame cutting.

Accordingly, the principal objects of this invention are to provide an improved method of and apparatus for eliminating such hardening and other objectionable change in the metallur- 50 gical structure of such severed steel surfaces by preventing the formation of the hardened zone or by reestablishing therein the desirable properties of the metal, during or immediately after the cutting operation, so that the cut section may 55 be used directly for structural purposes without

machining off hardened edges and without subsequent heat treatment or the customary furnace heat treatment of the entire piece of steel.

The above and other objects, as well as the novel features of this invention, will become more 5 apparent from the following description considered in connection with the accompanying drawing, in which:

Figs. 1 and 2 are side and end views, respectively, of an apparatus embodying this invention 10 and adapted for use in practicing the improved method;

Figs. 3 and 4 are side and end views, respectively, of a modified form of an oxy-fuel gas apparatus embodying this invention and adapted 15 for use in practicing a variation of the improved method; and

Fig. 5 is a side elevation similar to Fig. 1 showing an apparatus employing cutting and heating electrodes. 20

Ordinarily when the oxy-acetylene cutting flame (consisting of one or more high temperature gaseous heating jets and a gaseous oxidizing jet) progressively severs metal, such as a plate of high carbon steel or structural silicon steel, 25 the metal at the point of cutting attains a very high temperature which drops very rapidly at the moment the cutting flame leaves each successive point. This rapid temperature drop is due to the chilling or quenching effect of the 30 adjacent air and the adjoining mass of metal, and results in decided and objectionable changes in the physical properties of the metal along the cut or exposed surfaces, as set forth above.

In the flame cutting of such steels, the objects 35 of the invention are attained by what may be termed "localized heat treatment" applied, preferably during the cutting operation, directly to the flame cut surfaces and the metal adjoining the same, as by the localized application of one 40 or more relatively small high-temperature oxy-fuel gas flames.

In the preferred procedure of this invention the heat treating operation is integrated with the cutting operation. One or more oxy-acety- 45 lene or similar high-temperature heating flames are arranged so as to progressively follow the kerf as it is formed by the cutting flame and to impinge on the surfaces and edges exposed and thermally affected by the cutting operation. The 50 cutting flame and the heat treating flame or flames preferably move in unison relative to the work; and the distance between the cutting flame and the heat treating flame or flames as well as the intensity of the latter may vary considerably, 55

depending largely upon variable factors of the cutting operation such as the nature of the cutting medium, the composition and thickness of the work, the speed of cutting, etc.

5 The heat treating flame or flames are preferably located near and desirably immediately behind the cutting flame and, in this position, the intensity of the post-heating means and its spread along the kerf need only be sufficient to retard 10 rapid cooling of the cut surfaces and thereby prevent the otherwise sudden drop of their temperature to a point where the quenching action of the air and adjoining metal would be effective to objectionably harden the cut surfaces and 15 edges of the metal. These surfaces and edges then may cool gradually, so as to anneal the metal; that is to say, the metal, having been heated above the critical temperature, has additional localized heat applied thereto whereby it 20 is permitted to cool at such a slow rate as will result in a desirable softening or non-hardening effect on the steel. On the other hand, satisfactory results may be obtained when the heat treating flame or flames are applied to the cut 25 surfaces at a substantial distance behind the cutting flame, even beyond a point where the temperature of the cut surfaces has dropped to or below the recrystallization temperature. For example, the additional heat supplied to the cut 30 surfaces by the supplemental flame or flames may be sufficient to normalize the metal of such surfaces, i. e., to reestablish the desired metallurgical structure thereof by reheating them above a critical point, holding at that temperature 35 for a period, and then allowing cooling in air at room temperature.

In some instances, it is desirable to apply localized heat to the flame cut surface both immediately behind the cutting flame and at a substantial distance behind as just described; and with either or both of these arrangements it is sometimes also desirable to apply additional localized heat ahead of or alongside the cutting flame. In any event, the localized heat so applied may be of the same or graduated intensity 45 in a direction away from the cutting point, and may be either manually or mechanically propelled with the cutting flame over the work to be cut and the exposed and thermally affected 50 surface or edge to be treated.

While the kerf is being produced or after the cut has been completed, the two opposed surfaces thus exposed may be simultaneously locally and progressively heat treated, as described. 55 Such concurrent treatment or reconditioning of the metallurgical structure of both exposed surfaces saves both time and gas, especially if done during the cutting operation. In the latter case, the two surfaces are quite close together and, 60 since the heat applied thereto is more effectively utilized, less heat is required to recondition them than would be necessary later, after they are separated or have partially or completely cooled.

Usually it is desirable to progressively and locally heat treat the entire flame-cut edge or surface. However, certain situations arise in which it is desirable to apply the localized heat to soften only a portion of a hardened surface, to render such portion more readily workable 70 for a specific purpose; after which the worked portion may be restored to its original condition, as by re-hardening it.

The principles of this invention are especially adapted for use in the practice of severing metal 75 with an oxy-fuel gas cutting flame, such as the

oxy-acetylene cutting flame, but the invention is also useful when employing other high-temperature cutting agents, e. g., the electric arc with or without an auxiliary oxidizing agent such as oxygen. Similarly, the localized heat producing medium may consist of one or more electric arcs in combination with either a gaseous cutting flame or a cutting electric arc, the localized heat treatment being progressively applied to the cut surfaces behind the cutting point as the cut progresses and in such a manner that sufficient heat will be added to the metal to offset the effects of conduction of heat from the cutting flame or arc into the body of the metal and the cooling air quench which occurs in the cut surfaces immediately after they are cut. 15

It will be evident that the localized heat treatment may be utilized for annealing, tempering, normalizing or drawing, as required by the composition of the metal to establish therein the desired properties. For example, by locally applying the auxiliary source of heat in the immediate vicinity of the cutting point while cutting, the metal will absorb a considerable amount of heat by conduction and will then cool slowly to anneal the cut surface. Also, the metal of the cut surfaces may be similarly either tempered or normalized by locally applying the auxiliary source of heat to the cut edges at a considerable distance behind the cutting flame or along the 20 cut edges after they have cooled appreciably from the flame-cutting operation. In general, the localized heat treatment may be so adjusted and applied as to change or restore the metal surface treated to any desired or predetermined 25 condition; and it therefore will be understood that the procedure herein disclosed is subject to various changes without departing from the principles of the invention. 30

The accompanying drawing illustrates an apparatus for practicing the procedure just described. A preferred form of the apparatus, as shown in Figs. 1 and 2, may comprise a cutting blowpipe A of a common or usual design and heating units B and C rigidly connected therewith and so arranged in relation to the cutting blowpipe A that high temperature heating jets may be directed onto the work both ahead of and behind the cutting flame in alignment with the cut to be made. The high temperature heating jets from the units B and C are desirably aligned with the lower end or nozzle 10 of the cutting blowpipe A and are spaced at a relatively short distance therefrom, the distance being exactly determinable by the effect to be produced 45 by these jets. However, the high temperature heating jets do not necessarily need to be in alignment with the cutting jet, but may be arranged so as to direct heat on the general area both preceding and following the cutting flame 50 and the cut in the workpiece W. 55

The blowpipe A is provided with a mixing chamber and with both preheating gas and cutting oxygen passages of a construction common to cutting blowpipes, and also with the usual 60 type of control valves 11, 12 and 13, valves 11 and 12 being operable in governing the flow of preheating oxygen and acetylene respectively from intake connections and conduits 14 and 15 to a suitable mixer. The valve 13 controls the 65 supply of cutting oxygen and may have a handle 16 suitable for quickly turning on or shutting off the cutting oxygen jet. 70

A bracket 17 and frame 18 may be secured to the body of the blowpipe A in order to support a 75

gas supply conduit 19 for the units B and C, and a second bracket 20 may be adapted to embrace the conduit 19 and be rigidly secured to the frame 18 by a welded or other suitable joint. 5 Oxygen and acetylene supply pipes 21 and 22 respectively lead to a head 23 rigidly held at the lower end of the conduit and the oxygen and acetylene gases may be delivered through passages, which are conveniently arranged in the 10 head and controlled by valves 24, 24' and 25, 25' respectively, to mixing devices 26 and 27 of the type common to welding blowpipes.

From the mixing devices 26 and 27 the mixed oxygen and acetylene gases are then delivered 15 through stems 28 and 29 to manifolds within blocks 30 and 31 respectively, the blocks 30 and 31 being preferably secured to the blowpipe A at a substantial distance above the nozzle 10 and being disposed on each side of the blowpipe so as to be above the line of cut of the work. One 20 or more heating nozzles 32, 33 may be fixed to the manifold blocks 30 and 31 and extend downward to within a short distance of the work and desirably to a plane slightly above the end of the 25 nozzle 10.

In order to produce a sufficient amount of heat over a relatively large area of the work not only ahead of and behind the cutting jet but also at least partially alongside thereof, the manifold 30 blocks 30 and 31 are made arcuate in shape and three nozzles 32, 33 are connected with each of the blocks. The middle nozzle attached to each block is preferably aligned with the cutting nozzle 10 so that heat will be applied directly in line 35 with the cut ahead of the cutting jet and also along the edges E of the finished cut.

It will be appreciated that with the apparatus described the entire area immediately surrounding the newly formed cut may be raised to an 40 intermediate temperature, or to a degree of heat substantially below that produced by the cutting jet, which prevents sudden air quench of the metal from the high temperatures produced by the cutting flame and the oxidizing jet to room 45 or atmospheric temperature. As a result the edges E of the metal do not harden, or in the event that hardening does begin to take place, the post heating jets from the nozzles 33 prevent its continuation and restore the condition of the 50 metal substantially to the original state.

In order to further retard the rate of cooling of the metal following the cut, a refractory material R may be employed underneath the metal on either side of and closely adjacent the line 55 of the cut. Fire brick or other suitable non-fusing material when placed under the metal will assist in retaining the heat of the cutting flame as well as the heat from the blowpipe units B and C. The use of refractory material is 60 especially advantageous when the metal is relatively thick and subject to rapid conduction of the heat into the body thereof away from the cut edges, the refractory material serving in such instances to reflect and retain the heat in the 65 metal so that slow cooling will take place along the edges of the cut.

Another form of apparatus embodying this invention is shown in part in Figs. 3 and 4. This apparatus may comprise a cutting blowpipe A' 70 and only a post-heating unit C' which are rigidly connected together to move in unison. This unit may consist of a header 39 to receive and distribute the gaseous heating mixture to a group of nozzles 40, 41, 42 and 43 secured to the header 75 and forming part of the unit C' arranged to de-

liver heat behind the cutting blowpipe A' only. These nozzles may be desirably positioned so that two or more outer nozzles 40 and 43 direct jets alongside of the newly made cut, while two inner nozzles 41 and 42 direct jets at acute angles to the work so as to converge and form a very intense flame in the line of the cut. With this arrangement of the nozzles 41 and 42 it becomes possible to cut and after-heat relatively thick plates which would not be sufficiently heated by 10 a single flame to prevent hardening near the under surface or for the full depth of the plate. The converging jets from the nozzles 41 and 42 form an intense, penetrating flame which is capable of heating the sidewalls E' of the cut completely to the bottom thereof for most commercial sizes of plate. The heat produced by the nozzles of the unit C' may be adequate to heat 15 the area of the metal in the region of the cut to such a degree as to prevent sudden air quench without the aid of preheating nozzles arranged ahead of the cutting blowpipe A'. Whether or not a preheating unit need be employed is determinable by such factors as the thickness of the metal, the speed of cutting, the desired type 20 of treatment, the composition of the metal, etc.

While it is preferable to employ gaseous heating means to preheat and to after-heat the cut metal surfaces, it will be evident that electrical heating means such as electric arcs may be used 30 in some instances to preheat such surfaces or post-heat them, or a combination of the gaseous and electrical heating media may be used,—one for preheating and the other for post-heating.

The several types of apparatus here disclosed 35 are designed both to cut the metal and to prevent or counteract objectionable changes in the metallurgical structure of the surfaces exposed and thermally affected by the cutting operation. The flame or heat applied behind and in line 40 with the high-temperature cutting device extends into the kerf produced by the latter and retards the cooling of both surfaces of the cut. Such post-heating is desirably of considerably 45 less intensity than the heat at the cutting point and may be graduated, as by applying a series of flames of decreasing intensity along the kerf in a direction away from the cutting device.

Although several forms of apparatus embodying this invention are disclosed, it will be evident 50 that various changes may be made therein without departing from the principles of the invention.

I claim:

1. A method of cutting and treating ferrous 55 metals comprising flame-cutting the metal by locally heating successive portions of the metal to be cut, and simultaneously applying an oxygen-cutting jet to such locally heated portions; and concurrently with the cutting operation progressively reheating the successive cut portions after said portions have cooled to below the critical temperature, thereby raising the temperature of the cooled portions to counteract harmful metallurgical changes in the metal resulting from 60 the cutting operation.

2. The method of flame-cutting ferrous metals such as air-hardening and quench-hardening 65 steels and counteracting the thermal effects of the cutting operation on the flame-cut face and the edges adjoining the cut, comprising flame-cutting the metal by locally heating successive portions of the metal to be cut and simultaneously applying an oxygen jet to such locally heated portions; and progressively applying local 70

75

high-temperature heat to heat and thereby temper the flame-cut portions and the edges of the metal adjoining the successive cut portions after such edges and portions have partially cooled 5 to a point sufficiently below the recrystallization temperature to effect a tempering action.

3. A method of cutting ferrous metals so as to substantially counteract changes in the metallurgical structure of the cut and thermally-affected edges of the metal which comprises applying a high temperature heating and oxidizing jet to make the cut, applying sources of high temperature heat to the surface of the metal both ahead of and behind the cut, and moving 10 the heating and oxidizing jet and the sources of high temperature heat simultaneously relative to the surface of the metal.

4. The method of flame cutting metal and counteracting the thermal effects of the cutting 20 operation on the edges adjoining the cut, comprising locally heating successive portions of the metal to be cut; directing an oxygen cutting jet against the successive locally heated portions; applying a first source of local high temperature 25 heat progressively to the edges adjoining the successive cut portions after the edges have cooled to below the recrystallization temperature and subsequently applying a second source of local high temperature heat progressively to the 30 edges adjoining the successive cut portions to effect a tempering action after the edges have partially cooled from the application of said first source of heat.

5. The method of flame cutting metal and 35 counteracting the thermal effects of the cutting operation on the opposed edges adjoining the cut, comprising locally heating successive portions of the metal to be cut; directing an oxidizing cutting jet against the successive locally heated portions for cutting the metal; allowing the edges 40 adjoining the cut to partially cool; directing a plurality of converging heating jets within the kerf formed by the cutting jet; and exposing the successive portions of the opposed and partially 45 cooled edges of the kerf to the action of the converging jets.

6. An apparatus for flame-cutting ferrous metals such as air-hardening and quench-hardening steels and for counteracting the hardness 50 imparted to the edges during cooling from the flame-cutting operation, comprising means for projecting a flame-cutting jet against and progressively along a surface of the metal; and tempering means for directing localized high-temperature heat progressively along said surface to 55 portions of the metal thermally affected by said flame-cutting jet, said tempering means progressing in unison with said jet-projecting means and being located an appreciable distance behind said jet-projecting means so that the metal thermally affected by said flame-cutting jet cools to below the recrystallization temperature before being exposed to the action of the localized high-temperature heat from said tempering 60 means.

7. An apparatus for flame-cutting ferrous metals such as air-hardening and quench-hardening steels and for counteracting the hardness 65

imparted to the edges during cooling, comprising means for projecting a flame-cutting jet downwardly upon and progressively along the top surface of the metal; and post-heating means for directing localized high-temperature heat downwardly upon and progressively along the top surface portions adjoining the successive portions cut by said flame-cutting jet, said post-heating means progressing in unison with said jet-projecting means and being located an appreciable 5 distance behind said jet-projecting means so that the metal thermally affected by said flame-cutting jet cools to below the recrystallization temperature before being exposed to the action of the localized high-temperature heat from said 15 post-heating means.

8. Apparatus as claimed in claim 7 wherein said post-heating means comprises a heating unit having a plurality of nozzles for projecting localized high-temperature heat in a zone spaced a 20 substantial distance behind said jet-projecting means.

9. Apparatus as claimed in claim 7 wherein said post-heating means comprises nozzle means for directing localized high-temperature heat 25 against said top surface at a point an appreciable distance behind said jet-projecting means and in offset relation at one side of the line of cut.

10. An apparatus for cutting metal comprising high temperature oxidizing means to effect a cut, and metallurgical structure-restoring means comprising means for applying high temperature heat at a relatively short distance ahead of and behind said oxidizing means, said metallurgical structure-restoring means being separate 35 from the preheating means associated with said high-temperature oxidizing means.

11. An apparatus for cutting metal so as to prevent the hardening of metal along the edges 40 of the cut, which comprises a cutting blowpipe; and at least two oxy-fuel gas blowpipes arranged therebehind for introducing converging jets of high temperature gases against the newly cut edges of the metal.

12. An apparatus for cutting ferrous metal and for counteracting hardening of the metal along the edges of the cut, which comprises a cutting blowpipe movable with respect to the metal; and a plurality of means attached to said cutting 50 blowpipe in spaced relation thereto for applying high temperature heat along the newly-cut and partially cooled edges of the metal at successive substantially spaced intervals from the cutting blowpipe.

13. An apparatus for cutting metals and retaining good metallurgical structure therein, said apparatus comprising a cutting electrode movable along the surface of the metal, and at least one heating electrode attached a substantial 60 distance ahead of and at least one heating electrode attached a substantial distance behind said cutting electrode to apply high temperature heat to the surface of the metal in the region of the cut, whereby objectionable change in metallurgical structure is prevented.

ROBERT L. WAGNER.